

Feb. 18, 1936.

U. B. BRAY

2,031,204

## METHOD FOR PRODUCING LUBRICATING OIL

Filed Oct. 6, 1930

2 Sheets-Sheet 1

INVENTOR  
*Ulric B. Bray*  
BY  
*Philip Subkow*  
ATTORNEY.

Feb. 18, 1936.

U. B. BRAY

2,031,204

## METHOD FOR PRODUCING LUBRICATING OIL

Filed Oct. 6, 1930

2 Sheets-Sheet 2

INVENTOR.  
Ulric B. Bray  
BY Philip Lubkow  
ATTORNEY.

## UNITED STATES PATENT OFFICE

2,031,204

METHOD FOR PRODUCING LUBRICATING  
OIL

Ulric B. Bray, Palos Verdes Estates, Calif., assignor to Union Oil Company of California, Los Angeles, Calif., a corporation of California

Application October 6, 1936, Serial No. 486,725

15 Claims. (CL 196—13)

This invention relates to the production of lubricating oils from crude oils containing asphalt and wax.

It has been discovered that superior lubricating oil and asphalt can be obtained from crude oil by causing separation of the lubricating oil from the asphalt at temperatures below that at which deleterious changes are induced in the oil.

It has been found that if oil containing asphalt is heated in the presence of the asphalt, the latter catalyzes certain reactions in the oil which result in the destruction of those characteristics of the lubricating oils which are most desirable.

It has been found advisable to cause the separation of the asphalt from the oil by means of volatile solvents which are capable of dissolving the oil and any wax and which do not dissolve the asphalt. Such solvents are light petroleum fractions, such as casinghead gasoline and naphtha and also petroleum fractions normally gaseous at ordinary temperature and pressure. Other solvents which may be used are alcohol, ether, mixtures of alcohol and ether, acetone, etc. We prefer to use as our volatile solvent a petroleum fraction obtained by the rectification of natural gasoline. The fractions are composed in the main of propane and isobutane. A typical analysis of such a fraction is 6.72% ethane, 72.2% propane, 19.91% isobutane and 1.17% normal butane. It will be understood however that these merely illustrate the type of fractions used and the composition may vary. This fraction will hereinafter be referred to as propane for purposes of simplicity.

In order to cause extraction with this liquid fraction the solution is maintained at a pressure sufficient to maintain the propane liquid at ordinary temperatures. The fraction above described is liquid at ordinary temperatures at about 125 pounds pressure. The extraction of the oil from the asphalt at such pressure results in an asphalt substantially free of oil and a solution of oil in the liquid petroleum fraction. This solution contains substantially all the wax present in the crude oil.

It has also been found that oil containing asphalt and impurities such as wax may be first freed from the asphalt by a primary extraction with a light solvent such as the solvent described above and that the impurities such as wax may then be removed by the aid of a heavier solvent such as naphtha. By heavier solvent I mean one of higher boiling point than the light solvent previously described.

In order to avoid recompression to liquefy the

propane after separation from the oil, all or a substantial part of the propane is vaporized from the solvent oil solution under a pressure sufficiently high to permit condensation with the cooling medium available. The oil freed of this solvent is then treated to remove wax. The oil may also be purified by acid treatment, either before or after removal of the propane. By acid treatment I intend to include treatment with acid followed by the step of neutralization and/or clay treatment. Since the oil will be too viscous at the low temperatures necessary for the removal of wax, naphtha is added to the oil prior to the wax treatment. Naphtha may also be added prior to chemical treatment in order to avoid those difficulties usually encountered in chemically treating oils of high viscosity. By naphtha, I mean those petroleum fractions which vary from kerosene to light fractions of gasoline, preferably a gasoline-like fraction having a specific gravity of about 55° A. P. I. and a boiling range of about 200–300° F. Instead of naphtha I may use other solvents or diluents, for instance, benzol, alcohols such as methyl, ethyl, propyl, butyl alcohol or mixtures of the same, ketones such as acetone or di-ethyl ketone, chlorinated light hydrocarbons such as dichlorethylene, trichloroethylene or the like, or mixtures of benzol with acetone or other ketones, or mixtures of benzol and butanol or other alcohols.

In addition to the power which the naphtha has of reducing the viscosity of the asphalt-free oil, it also is used as an extracting medium for wax or other material whose presence is deleterious in a finished, high grade lubricating oil. The naphtha if used in sufficient quantities at low temperature acts as a solvent for the oil during the removal of the wax or other impurities in a manner similar to the action of the propane solution during the removal of the asphalt. By regulating the quantity and temperature substantially oil free wax may be precipitated. In comparing their volatility and specific gravity, the propane is considered to be the light solvent and the naphtha is the heavier solvent. An advantage in using both light and heavy solvents resides in the fact that the dewaxing may take place in the presence of the heavier solvent after the lighter, more volatile solvent has been removed.

The crude oil containing asphalt and wax is first topped to a temperature of about 600–625° F. to remove the gasoline, kerosene and all or a portion of the light lubricating oil, and the topped residuum is then treated by the process herein-after described.

It is, therefore, an object of my invention to produce lubricating oil from oil containing asphalt and wax by mixing this oil with a light solvent, said solvent being capable of separating the oil and wax from the asphalt, removing substantially all the solvent from the oil and wax, adding a heavier solvent such as naphtha to the oil and wax substantially free of the light solvent, and subsequently dewaxing the oil in the presence of the heavier solvent.

It is a further object of my invention to produce lubricating oil from the type of oil above described by mixing this oil with a volatile solvent under pressure thereby separating the asphalt from the oil and wax, removing at least a substantial portion of the solvent from the oil and wax under pressure, adding naphtha to the oil and wax substantially free of the solvent, and subsequently dewaxing the oil in the presence of the naphtha.

Another object of my invention is to include chemical treatment of the oil in the processes outlined above, said chemical treatment being either before or after the removal of the propane from the asphalt free oil.

The process will be more adequately understood by reference to the drawings which show schematic arrangements of the apparatus to carry out the process described herein.

Fig. 1 is a schematic arrangement of apparatus in which the oil is first made asphalt free and then is chemically treated under pressure following which the propane is distilled off under pressure and then the oil is dewaxed in the presence of naphtha.

Fig. 2 is a schematic arrangement of apparatus in which the oil is first made asphalt free and then a substantial portion of the propane is removed under pressure, following which the remaining propane is removed under released pressure; the oil is chemically treated and finally dewaxed in the presence of naphtha.

Referring more particularly to Fig. 1, the topped residuum which has been produced from the selected crude by a suitable topping operation, preferably at 600-625° F., is stored in tank 1 from which it is sent by pump 2 through line 3 to T 4 where it meets liquid propane containing a small amount of oil coming through line 5. The mixture of propane and residuum pass from T 4 through mixing coil 6 into decanter 7, where the asphalt in the topped residuum is precipitated and settles rapidly as a slurry. From the bottom of decanter 7, the asphalt slurry is sent by pump 8 through line 9 to line 10 where fresh liquid propane is introduced by pump 11 from liquid propane storage 12. The asphalt slurry and fresh liquid propane are sent through mixing coil 13 into decanter 14.

The asphalt-propane slurry from the bottom of decanter 14 is drawn off through expansion valve 15 and line 16 and discharged at a lower pressure into coil 17 set in furnace 18, where heat is supplied for the purpose of vaporizing the propane and melting the asphalt. The heated materials are passed from coil 17 through pressure reduction valve 19 into evaporator 20 which operates at a lower pressure. Superheated steam is introduced via 21 into evaporator 20 to supply additional heat and to reduce the asphalt to proper specifications as to fire and flash points. The asphalt is taken from the bottom of evaporator 20 and sent through the rundown line 21 by pump 22 to asphalt storage 23. The vapors in evaporator 20 pass through mist extractor 24 and are then

sent through line 25 to cooler 26 and to separator 27. The uncondensed propane from separator 27 is sent through line 28 to line 29 and to propane compressor 30 where its pressure is raised to the pressure in the high pressure system. The propane is then sent through line 31 to propane cooler 32 where it liquefies and runs down into propane storage tank 12.

The overflow from decanter 14, containing the oil and wax washed from the asphalt slurry taken from decanter 7, is sent by pump 33 through line 5 to T 4 where it is mixed with the topped residuum and sent into decanter 7 as explained above. The overflow from decanter 7, consisting of propane and lubricating oil stock, is sent through pump 35 and line 36 to turbulence or mixing coil 37 where the acid and alkali treatment of the extracted lubricating oil stock begins. The countercurrent washing of the precipitated asphalt illustrated by the above method of operating decanters 7 and 14 may be extended to as many steps as desired, but in general two decanters giving two countercurrent washings will be sufficient to give an asphalt of satisfactory wax content.

To the propane solution of extracted lubricating stock, acid from tank 38 is added through line 39 by means of pump 40. The propane solution and acid are forced by the pumps 35 and 40 through mixing coil 37 into decanter 41 where the sludge is allowed to settle. The acid sludge is removed via 42. The oil containing some acid flows from decanter 41 through line 43 by pump 44 into decanter 45 where water is introduced as a spray through line 46, from water storage 47 through pump 48 and valve 49. The water washed oil overflows from decanter 45 and is sent by pump 50 to line 51 where caustic soda solution is introduced by pump 52 through line 53 from tank 54. The wash water is removed from decanter 45 via 55. The mixture of oil solution and aqueous alkali solution is forced through mixing coil 56 into decanter 57 where the spent caustic solution separates from the propane solution of the oil and is withdrawn via 58.

The overflow from decanter 57 goes through line 59 via pump 60 to decanter 61 where water is introduced as a spray through line 62 and valve 63 by pump 48. The continuous and rapid treatment of lubricating oil stocks as described above is made possible by operating in the presence of propane, and is a distinct advantage of the process. Wash water is removed from decanter 61 via 67. The neutralized and water washed oil solution overflowing from decanter 61 is carried by pump 64 through line 65 to the surge tank 66 which acts as a reservoir between the acid treating and propane recovery operations.

Decanters 7, 14, 41, 45, 57 and 61 together with propane storage 12 and surge tank 66 are maintained at the same pressure by means of equilibrium lines 70 controlled by valves 71. The pressure that is maintained is sufficient to keep the solvent in liquid state at ordinary temperatures. For the solvent given above, this is about 125 lbs. per sq. in. at about 70° F.

The treated oil solution in tank 66 is sent through valve 75, line 76 and pump 77 into the high pressure exhausting column 80, which preferably consists of plates 81 carrying closed steam coils 82. The pressure in 80 is maintained at a sufficient point to cause condensation in condenser 82 without applying additional pressure in the condenser.

As the oil in propane solution travels down col-

umn 80, the propane is vaporized, passes through mist extractor 83 and exits through line 84 to line 31 from which the vapors pass to cooler 32 where they are liquefied and allowed to run down into liquid propane storage 12. The bottoms from column 80 consist of treated lubricating oil containing a small amount of dissolved propane. These bottoms are drawn off through pressure release valve 85 and line 86 into which naphtha from tank 87 is introduced through pump 88 and line 89 controlled by valve 90. The naphtha and oil pass through mixing coil 91 into blending or storage tank 92. The use of additional heat or agitation in tank 92 may or may not be necessary.

15 The blended oil-naphtha mixture is then passed from tank 92 through line 93 by pump 94 into cooling chamber 95 where the mixture is chilled at a proper rate to a suitable dewaxing temperature by means of cooling coil 96. The chilled mixture passes through line 97, pump 98 and valve 99 into centrifuge 100 driven by motor 101. The dewaxed oil solution discharged from the center of the centrifuge is then sent through line 102 to dewaxed naphtha-oil storage 103.

25 The dewaxed oil solution is sent from storage 103 through pump 104 and line 105 to heat interchanger 106 where heat is absorbed from naphtha vapors and steam from column 107 as described below. Leaving heat interchanger 106, the oil-naphtha mixture passes into exhausting column 107 in which open steam may be introduced via 108. The bottoms from column 107 consist of acid treated and dewaxed oil which has been reduced by steaming to flash and fire characteristics determined in the main by the extent of topping of the crude residuum stored in tank 1. The bottoms from column 107 are removed via line 109 and may be cooled by heat exchange in heat exchanger 110 in a manner to be described below. The oil leaving the heat exchanger 110 is sent by line 111 to treated oil storage 112, from which it may be sent to a clay treating plant or the like.

35 The overhead from column 107 is sent through mist extractor 115 and then to heat exchanger 106 by line 116 where heat is imparted to the incoming naphtha-oil solution as described above. The partially condensed overhead vapors next pass from heat exchanger 106 through line 117 to cooler 118 and then to separator 119. The naphtha condensate in separator 119 is sent by pump 120 through line 121 to naphtha storage 87. The uncondensed propane from separator 119 passes through line 122 to line 29 where it is admitted to the suction of propane compressor 30, which discharges into the high pressure propane vapor line 31 as described above.

45 The wax discharged from the centrifuge through line 125 is melted by hot water introduced through line 126. The hot water and melted wax in line 125 pass into wax separator 127 from which the wax is removed via 128 into storage 129.

55 The water settling in wax separator 127 is withdrawn through line 130 by pump 131 into water storage 132 from which it may be withdrawn through line 133 by pump 134 into line 126 which passes through heat exchanger 110. Before recycling into pipe 125 the water is thereby heated by heat exchange in 110 with the bottoms from column 107 which are correspondingly cooled.

65 Referring more particularly to Fig. 2, this embodiment relates to the aforesaid process in which a modification is made whereby the chemical treatment takes place in the absence of substan-

5 tial quantities of the solvent due to a preliminary removal of the solvent from the oil and wax.

6 The topped residuum from tank 1 is carried through line 2 to pump 3 and thence to line 4 where it meets a propane solution of lubricating oil coming through line 15. The propane and residuum pass through the turbulence or mixing coil 5 into decanter 6. The asphalt in the residuum is precipitated by the propane and settles to the bottom of decanter 6. The asphalt-propane slurry from decanter 6 is passed through pump 8 in line 7 to line 9 where fresh liquid propane from storage 10 coming through pump 10 and line 9 is added and the mixture then passes through mixing coil 11 into decanter 12. In this second extraction the asphaltic bodies are freed of substantially all the oil and wax contained in the asphaltic material. The mixed oil and propane is passed through line 13, pump 14 and line 15 into line 4 for treatment as previously described. Decanters 6 and 12 and tank 10 are connected by pressure equalizing lines 16 controlled by valves 17. The pressures in 6, 12, and 10 are sufficiently high to maintain the solvent in liquid condition. For the solvent described above the pressure is about 125 lbs. at about 70° F.

10 15 20 25 30 35 40 45 50 55 60 65 70 75

The asphalt slurry from decanter 12 is drawn off through the pressure release valve 17 and sent through to coil 18 positioned in furnace 19 where sufficient heat is supplied to cause vaporization of the propane and to melt the asphalt. The heated mixture of asphalt and propane is now sent through line 20 to the evaporator 21 where superheated steam is introduced via 22 in order to complete the vaporization of the propane and reduce the asphalt to satisfactory flash and fire specifications. The pressure in the vaporizer 21 is substantially atmospheric. The overhead from the evaporator 21 is sent through line 23 to condenser 24 and into separator 26 via line 25. The uncondensed propane from separator 26 is carried through line 27 to propane compressor 28.

25 30 35 40 45 50 55 60 65 70 75

The compressed propane from compressor 28 passes through line 29, line 30, pump 31 and line 32. It is then condensed in condenser 33, the condensed propane passing to storage 10. The condensed oil which has been entrained in the asphalt slurry and vaporized in 21 is withdrawn through 26a and the condensed steam through 26b. The reduced asphalt is sent through line 35 to asphalt storage 36 via pump 34.

35 40 45 50 55 60 65 70 75

The clear overflow from decanter 6 containing a higher percentage of dissolved lubricating oil passes through line 37, pump 38 and line 39 to heat exchange 40 where its temperature is raised somewhat before passing through line 41 into high pressure evaporator or dephlegmator 42. The object at this point is to add sufficient heat to the liquid propane solution to cause substantially complete vaporization of the liquid propane at a pressure somewhat higher than that being maintained in cooler 33. Heat may be applied at this point by any desired means, but in the drawing a steam coil 43 is shown in the bottom of the dephlegmator. The pressure in 42 is maintained by controlling the temperature in the dephlegmator by proper manipulation of valve 44a in vapor line 44. The pressure in 42 is maintained at a sufficient point to cause condensation in the condenser 33 without applying additional pressure in the condenser. When heat is applied to the propane solution under pressure, the propane vaporizes and travels through 44, line 30, line 32 and cooler 33 where the propane 75

condenses and passes back to liquid propane storage 10. The temperature and pressure employed in dephlegmator 42 will determine to what extent the propane is completely removed from the oil remaining in the bottom of the dephlegmator, but in general there will be sufficient propane remaining in the oil drawn from the bottom of the dephlegmator to justify a further recovery of propane under reduced pressure.

10 The oil leaving the dephlegmator 42 then passes through the pressure release valve 45 and line 46 into the low pressure dephlegmator 47. Additional heat may or may not be needed at this point, but in order to insure more complete recovery of propane, steam may be introduced into dephlegmator 47, via 48. The overhead from dephlegmator 47 passes through line 49 to condenser 50 and then into separator 51. The uncondensed propane from separator 51 is carried 15 through line 52 to propane compressor 53. Compressor 53 raises the pressure of the propane to that being carried in the high pressure evaporator 42 and the compressed propane is then passed 20 through line 20 going eventually to propane storage 10 as described above. The water condensed in 51 is withdrawn through line 55 and any oil evaporated in 47 and condensed in 50 is withdrawn through 54.

The hot lubricating oil stock in the bottom of 30 the low pressure dephlegmator 47 is passed through line 56 by pump 57 to heat exchanger 48 where it imparts heat to the propane solution in line 41 as described above. Leaving the heat exchanger 48 the oil passes through line 59 to 35 lubricating oil stock storage 60 from which it is withdrawn by pump 61.

If it is desired to chemically treat the lubricating stock in the presence of naphtha, the lubricating oil stock passing through valve 62 in 40 line 66 is admixed with naphtha passing from tank 63 via pump 64 by proper operation of valves 62 and 65 and 85. The mixture of oil and naphtha passes through line 66 to agitator 67 where it is treated with sulfuric acid received from 45 tank 68 by operation of pump 69 and valve 70. The decanted oil-naphtha solution is drawn off through valved draw off lines 72, and carried through 73 into agitator 74. The acid sludge is withdrawn via draw off line 71. The oil is then 50 washed with water, treated with caustic and again washed in 74, in separate stages with intermediate withdrawal of water and caustic. Water is supplied from tank 75 by operation of pump 76 and valve 77, and caustic is supplied from tank 78 by operation of pump 80 and valve 81. The water and caustic are separately withdrawn via 82. The treated oil in agitator 74 is drawn off through valve 83 and sent through line 86 by pump 87 to refrigeration machine 88. In case 60 additional naphtha is needed for the dewaxing operation, this may be supplied through line 84 by opening valve 85.

If it is not desired to chemically treat the lubricating oil stock in the presence of naphtha, the oil leaving storage 60 is passed directly through valve 62 and line 66 into agitator 67 with valve 65 being closed. After treatment in the two agitators, the oil passes through valve 83 in line 86 where a suitable quantity of naphtha for use in 70 the dewaxing operation is added from naphtha storage tank 63 by opening valve 85. The oil-naphtha solution is then sent into chilling vessel 88 via pump 87. The chilling vessel may be any type of refrigeration equipment. As a specific example this machine consists of expansion

coil 89, compressor 91, cooling coils 92, tank 93 and expansion valve 98. The refrigerant may be ammonia or a volatile product such as is used in the extraction operation described above. The operation of this refrigerating equipment will be understood by those skilled in the art.

The chilled solution is taken from the cooling vessel 88 by line 94 and passed into centrifuge 95 of conventional design. Wax is discharged from the centrifuge through line 95a. The discharged wax may be worked up by any convenient means for the recovery of naphtha and oil. Dewaxed naphtha solution is discharged from the centrifuge through line 96 into surge tank 97 and is sent through pump 98 and line 99 into heat exchanger 100 where it absorbs heat from condensing naphtha vapors coming through line 106, as explained below. Instead of interchanging the cold naphtha solution with naphtha vapors as in 100, the cold naphtha solution may be interchanged with the incoming naphtha solution in line 86 before the naphtha solution is sent to chilling vessel 88.

The naphtha solution leaving heat exchanger 100 passes through line 101 to coil 102 in furnace 19 and thence into evaporator 104 via line 103. Sufficient heat is absorbed in coil 102 to raise the temperature sufficiently to distill the naphtha with aid of steam introduced via 105 into evaporator 104. The naphtha is taken overhead through line 106 to heat exchanger 108 and to condenser 108 via line 107. The condensed naphtha is sent to separator 109 and then passes through line 110, pump 111 and line 112 into naphtha storage tank 63. The condensed steam exits through 110a. The bottoms from evaporator 104, consisting of dewaxed oil are now passed through line 112, pump 114, cooler 115 and line 116 into acid treated dewaxed oil storage tank 117.

It is to be understood that the above is merely illustrative of preferred embodiments of the invention of which many variations may be made by those skilled in the art without departing from the spirit thereof.

I claim:

1. A method of separating asphalt and wax from oil containing the same which comprises mixing said oil with a liquefied volatile solvent, separating said asphalt from the liquefied solvent, oil and wax, separating substantially all of said solvent from the oil and wax, adding naphtha, to cause separation of wax from the oil-naphtha solution, removing the wax from the oil and naphtha and subsequently removing the naphtha from the oil.

2. A process for the production of lubricating oil from an oil containing asphalt and wax which comprises mixing said oil with liquid propane, separating the asphalt from the oil, wax and liquid propane, acid treating the oil, wax and liquid propane, separating the propane from the acid treated oil and wax, adding a wax extracting solvent to the acid treated oil and wax, separating the wax from the oil and wax extracting solvent and separating the wax extracting solvent.

3. A process for the production of lubricating oil from an oil containing asphalt and wax which comprises mixing said oil with liquid propane, separating the asphalt from the oil, wax and liquid propane, acid and alkali treating the oil, wax and liquid propane, separating the propane from the treated oil and wax, adding a heavy solvent to the treated oil and wax, separating the wax from the oil and heavy solvent and separating the heavy solvent from the oil.

4. A process for the production of lubricating oil from an oil containing asphalt and wax which comprises mixing said oil with liquid propane under superatmospheric pressure to separate asphalt, separating the asphalt from the oil, wax and liquid propane under superatmospheric pressure, separating the propane from the oil and wax under superatmospheric pressure, adding naphtha to the oil and wax, cooling the naphtha, oil and wax sufficiently to precipitate the wax, separating the precipitated wax from the oil and naphtha and separating the naphtha from the oil.

5. A process for the production of lubricating oil from an oil containing asphalt and wax which comprises mixing said oil with liquid propane, separating the asphalt from the oil, wax and liquid propane, separating the liquid propane from the oil and wax, adding a heavy solvent to the oil and wax, acid treating the oil, wax and heavy solvent and separating the heavy solvent from the acid treated oil and wax.

6. A process for the production of lubricating oil from an oil containing asphalt and wax which comprises mixing said oil in liquid propane under superatmospheric pressure to separate asphalt, separating the asphalt from the oil, wax and liquid propane, separating the propane from the oil and wax under superatmospheric pressure, chemically treating the oil and wax, adding a heavy solvent to the oil and wax, separating the wax from the oil and heavy solvent and separating the heavy solvent from the oil.

7. A process for the production of lubricating oil from an oil containing wax which comprises mixing said oil with liquid propane, acid treating the oil, wax and liquid propane, separating the propane from the acid treated oil and wax, adding naphtha to the acid treated oil and wax, separating the wax from the oil and naphtha and separating the naphtha from the oil.

8. A process for the production of lubricating oil from an oil containing wax which comprises mixing said oil in liquid propane under superatmospheric pressure, acid treating said oil, wax and liquid propane, separating the propane from the acid treated oil and wax under superatmospheric pressure, adding naphtha to the acid treated oil and wax, cooling the naphtha, oil and wax, separating the wax from the cooled oil and naphtha and separating the naphtha from the oil.

9. A process for the production of lubricating oil from an oil containing wax which comprises mixing said oil in a volatile solvent, acid and alkali treating said oil, wax and volatile solvent, separating the volatile solvent from the treated oil and wax, adding naphtha to the treated oil and wax, cooling the naphtha, oil and wax, separating the wax from the cooled naphtha and oil and separating the naphtha from the oil.

10. A method for the separation of asphalt and wax from oil which comprises commingling said oil with a normally gaseous liquid hydrocarbon solvent to separate asphalt, separating the asphalt from the oil and wax dissolved in said sol-

vent, removing the solvent from the oil and wax, adding a heavier solvent to the oil and wax, cooling the heavy solvent solution of oil and wax to precipitate wax and separating the precipitated wax from the oil and heavy solvent.

11. A method for the separation of asphalt and wax from oil which comprises commingling said oil with a normally gaseous liquid hydrocarbon solvent to separate asphalt, separating the asphalt from the oil and wax dissolved in said solvent, separating the solvent from the oil and wax, dissolving said oil and wax in a heavy hydrocarbon solvent, cooling said heavy hydrocarbon solution of oil and wax to precipitate wax and separating the precipitated wax from the oil dissolved in said heavy hydrocarbon solvent.

12. A method for the separation of asphalt and wax from oil which comprises commingling said oil in a liquefied normally gaseous hydrocarbon solvent, the major portion of which is propane to separate asphalt, separating the asphalt from the oil and wax dissolved in said solvent, removing the solvent from the oil and wax, dissolving said oil and wax in a heavier solvent than said first mentioned solvent, cooling the oil and wax dissolved in said heavy solvent to precipitate wax and separating the precipitated wax from the oil dissolved in said heavy solvent.

13. A method for the separation of asphalt and wax from oil which comprises commingling said oil in a liquefied normally gaseous hydrocarbon solvent, the major portion of which is propane, to separate asphalt, separating the asphalt from the oil and wax dissolved in said solvent, separating the solvent from the oil and wax, dissolving said oil and wax in naphtha, cooling the naphtha solution of oil and wax to precipitate wax and removing the precipitated wax from the oil dissolved in naphtha.

14. A method for the separation of asphalt and wax from oil which comprises commingling said oil with a liquefied normally gaseous hydrocarbon solvent, containing a major portion of hydrocarbons having less than four carbon atoms to separate asphalt, separating the asphalt from the oil and wax dissolved in said solvent, separating said solvent from the oil and wax, dissolving said oil and wax in naphtha, cooling the naphtha solution of oil and wax to precipitate wax and separating the precipitated wax from the oil dissolved in naphtha.

15. A method for the separation of asphalt and wax from oil which comprises commingling said oil with a liquefied normally gaseous hydrocarbon solvent containing a major portion of hydrocarbons having less than three carbon atoms to separate asphalt, separating the asphalt from the oil and wax dissolved in said solvent, removing the solvent from the oil and wax, dissolving said oil and wax in a heavier hydrocarbon solvent than said first mentioned solvent, cooling the heavy solvent solution of oil and wax to precipitate wax and separating the precipitated wax from the oil dissolved in said heavy solvent.

ULRIC B. BRAY. 65